

July 13, 1965

R. D. CULBERTSON ET AL

3,193,920

## PRESSURE SEALING OF PLATED ENVELOPE SECTIONS

Original Filed Aug. 17, 1959



Fig. 1



Fig. 2



Fig. 3

INVENTORS.  
ROBERT D. CULBERTSON  
RUSSELL C. MCRAE  
BY HARVEY C. WARNER  
*Robert W. Ditts*  
*Leon F. Herbert*  
ATTORNEYS

1

3,193,920

## PRESSURE SEALING OF PLATED ENVELOPE SECTIONS

Robert D. Culbertson, San Jose, Russell C. McRae, Santa Clara, and Harvey C. Warner, Belmont, Calif., assignors to Eitel-McCullough, Inc., San Carlos, Calif., a corporation of California  
Original application Aug. 17, 1959, Ser. No. 834,219.  
Divided and this application Nov. 13, 1962, Ser. No. 237,208

4 Claims. (Cl. 29—492)

This application is a division of our copending application Serial No. 834,219, filed August 17, 1959.

This invention relates to an electron tube and more particularly to an electron tube having a pressure seal and to a method of and a means for making such a seal. The term "pressure seal" is defined for use herein as a permanent vacuum-tight seal obtained by the application of pressure at temperature below the melting point of any of the materials in the seal.

With the introduction of high alumina ceramic electron tubes, various types of pressure seals were developed to seal ceramic to ceramic or ceramic to metal. None of these types of seals are effective in sealing two parts of a miniature electron tube, especially when the tube dimensions are in the order of one-half inch long and one-quarter inch in diameter. In pressure sealing a miniature diode that requires at least three electrical leads and is limited to two ceramic ring insulators, the electrical lead, which is in the form of a ring and positioned between the two ceramics, is required to be made of hard metal such as Kovar so that it will not deform under sealing pressure destroying the metal to ceramic bond, as well as making it difficult to obtain accurate electrical spacing. The art of pressure welding two pieces of metal teaches that hard metals require larger pressures for pressure welding than softer metals. The pressure required to weld Kovar is too high and not practical in the fabrication of a miniature tube.

In this application Kovar refers to metal alloys comprising primarily iron, nickel and cobalt with some manganese and having a coefficient of thermal expansion approximately  $5 \times 10^{-6}$  per degree centigrade.

It is an object of the present invention to provide an electron tube with a pressure seal between two pieces of hard metals.

It is another object of the present invention to provide a pressure sealing method between hard metal surfaces which do not require optical flat joining surfaces.

It is yet another object of the present invention to provide a pressure seal, a method of and a means for making such seal between hard metal rings in an electron tube.

In one embodiment the invention involves making hard metal pressure seals for electron tubes by plating the hard metal sealing rings with a soft ductile metal. A soft ductile metal sealing gasket is placed between the two soft metal clad surfaces on each of the hard metal rings. Force is applied to the hard metal rings until the gasket yields and deforms. In so doing the gasket adheres to the plated surfaces.

The invention possesses other objects and features of advantage, some of which, with the foregoing, will be set forth in the following description of the invention. It is to be understood that the invention is not limited to the disclosed species, as variant embodiments thereof are contemplated and may be adopted within the scope of the claims.

Referring to the drawings:

FIGURE 1 is a sectional elevation of a typical die press fixture, through which pressure is applied to the sealing rim of an electron tube.

2

FIGURE 2 is an enlarged view of the sealing rim of an electron tube before pressure is applied.

FIGURE 3 is a sectional elevation of the sealed electron tube.

Referring now to the drawings and to FIGURE 1 in particular, there is shown an electron tube in two sections which are to be sealed together. The two sections are cathode section 12 and an anode section 14. The cathode section 12 is suspended within an axial well 16 formed in a ram 18. The ram 18 and a die 20 form a die press fixture. The cathode section is held by a wire 22 which is suspended through an aperture 24 in the ram 18. The end of the wire 22 within the well 16 is fixed to a sealing means 26 which is a metallic plate joined to a ceramic cylinder 28 of the cathode section 12 by means of a conventional ceramic-to-metal bond. Wire 22 may be fixed to sealing means 26 with soft solder. The wire is then passed through aperture 24 and the cathode section is drawn up tight against the ram 18. The wire's free end protruding from the ram is bent to hold the cathode section in place. On the other end of the ceramic cylinder 28 is bonded a terminal sealing ring 30 preferably made of Kovar. The terminal sealing ring 30 is plated with a soft, highly ductile metal 32 such as oxygen-free, high conductivity copper, which in this embodiment is plated on both sides of the Kovar, as shown, although it is actually necessary to plate only the side of the Kovar to be pressure sealed. The plating is preferably between .001 and .002 inch thick and the ring 30 is about .010 inch thick. A cathode 33 with an emitting surface 34 coplanar with the plated 32 surface of the terminal ring 30 is mounted thereto.

The anode section 14 is similar to the cathode section in that sealing means 26' formed into a cup-shaped metal section is sealed to a similar ceramic cylinder 28' and a terminal ring 30' is joined to the other end of the ceramic cylinder 28' by means of a conventional ceramic-to-metal bond. Ring 30' is also made of a hard metal such as Kovar. The sealing means 26' is the anode with a face 35 coplanar with the plated 32' surface of the terminal sealing ring 30'. Similarly to ring 30, the ring 30' is also copper plated as represented by plated layers 32'. The anode section 14 fits into the die 20 with the ceramic section 28' disposed within a bore 34 of the die 20 and the terminal sealing ring 30' bearing on a shoulder formed by a larger bore 36 into which is disposed the ram 18.

The pressure seal is formed between the two rings 30 and 30' by first cleaning the sealing surfaces which are the copper plated surfaces 32 and 32' which face each other and cleaning a soft highly ductile metallic sealing gasket 38 made of the same material as the plated surfaces 32 and 32', and in this embodiment being oxygen free, high conductivity copper, all being cleaned with a standard acid process. The two sections 12 and 14 and the copper gasket 38 are afterward wet-hydrogen fired at approximately 800° C. to anneal, degas and remove carbon residue. The two sections 12 and 14 are assembled to the ram 18 and die 20, as shown in FIGURE 1, with hard metal washers 40 and 40' disposed between the terminal sealing ring 30 and the ram 18 and between the terminal sealing ring 30' and the die 20, clearly shown in FIGURE 2. The hard metal washers 40 and 40' are preferably made of Kovar and are used to prevent the copper plating on the rings 30 and 30' adjacent the ram and the die from adhering thereto. The sealing gasket 38 is placed on the plated layer 32'. Also on the plated layer 32' is placed a hard metal spacer washer 42, also preferably made of Kovar. The washer 42 is thinner than the sealing gaskets 38, and it is used to limit the space between the anode face

35 and the emitting surface 34. The ram 18 and die 20, along with the tube are enclosed in a vacuum envelope (not shown) and vacuum fired between 600° and 700° C. The vacuum pressure is reduced to  $1 \times 10^{-4}$  mm. of mercury at this temperature. An electrical resistance coil 50 may be used for the vacuum firing process. The coil 50 is powered by a suitable power supply 52 and controlled by a variable resistor 54. The tube is processed in a standard manner during the vacuum firing.

After vacuum firing and still maintaining a high vacuum, the ram 18 is then forced against the die 20 by a press 56. A pressure of about 25000 p.s.i. on the sealing gasket 38 is applied for 2 to 5 minutes at a temperature of about 500°-600° C. The pressure, temperature, time combination can be varied somewhat as long as the temperature is below the melting temperature of copper and above the annealing temperature; the lower the temperature, the greater the pressure and time requirement and vice versa. The sealing gasket 38 is extruded under this pressure causing it to adhere to the layers 32 and 32' and a like metal to like metal (copper to copper) seal is made. The spacer washer 42 limits the spacing between the rings 30 and 30' and also prevents the sealing gasket from extruding into the tube and making an electrical short.

Although the seal is a copper-to-copper seal, rings 30 and 30' made entirely of copper are not practical since copper will extrude and deform during the pressing operation. This deformation of the copper would destroy the vacuum tight bond with the ceramic. A ring 30 and 30' made of hard metal such as Kovar does not deform in making the seal and therefore retains the vacuum tight bond with the ceramic. Further, if copper were used, the spacer washer 42 would imbed itself in the terminal sealing rings and no longer serve the purpose of fixing the cathode, anode spacing.

FIGURE 3 shows the sealed electron tube. The tube is shown in cross-section in order to illustrate what happens to the copper gasket 38 after pressure is applied. The copper flows under pressure and is prevented from flowing into the vacuum envelope by the spacer washer 42. The copper in thus flowing adheres to the adjacent copper plating strips 32 and 32'.

What is claimed is:

1. A method of pressure sealing two vacuum envelope sections, said sections each having a hard metal sealing ring protruding outwardly from each of said sections forming rims, said sealing rings being plated with a soft ductile metal, said method comprising the steps of placing a hard metal spacer ring on said plated surface of one of said sealing rings substantially coaxially with said one of said sealing rings, placing a soft metal gasket fabricated from the same material as said soft ductile plating and having a thickness greater than said spacer ring on a plated surface of said one of said sealing rings substantially coaxially with and exterior of said spacer ring, placing a plated surface of the other of said sealing rings on said

5 gasket substantially coaxially with said spacer ring, forming a vacuum around said sections, heating said rings and gasket to a temperature below the melting temperature and above the annealing temperature, and applying pressure to said rims on both of said sealing rings to compress said sealing gasket causing it to adhere to said plated surface of said rings.

2. A method of pressure sealing two copper plated sealing rings disposed on each of two vacuum envelope sections, said sealing rings being made of a metal substantially harder than said copper plating and protruding outwardly from said envelope sections forming rims, the method comprising the steps of placing a spacer ring on a copper plated surface of one of said sealing rings substantially coaxially with said plated surface, said spacer ring being made of a metal substantially harder than copper, placing a copper gasket having a thickness greater than said spacer ring on said copper plated surface of said one of said sealing rings substantially coaxially with and exterior of said spacer ring, placing a copper plated surface of the other of said sealing rings on said copper gasket, forming a vacuum of about  $1 \times 10^{-4}$  of mm. of mercury around said sections of said electron tube, vacuum firing said two sections between about 600° and 700° C., and applying pressure to said rim on both of said sealing rings to compress said copper gasket causing it to adhere to the plated surface of said rings but not deforming said spacer ring.

3. A method of pressure sealing two hard metal sealing rings disposed on each of two envelope sections, the method comprising the steps of plating each sealing surface on each of said sealing rings with a soft ductile metal, placing a soft ductile metal gasket which is formed from the same type as said ductile plating on a plated surface 35 of one of said sealing rings substantially coaxially therewith, placing the plated surface of the other sealing ring adjacent the metal gasket so that the metal gasket is located intermediate the plated surfaces of the two sealing rings, firing said two sections at a temperature below the melting temperature and above the annealing temperature of said metal gasket and said soft ductile plating, and applying pressure to said sealing rings to compress said sealing rings together thereby extruding said metal gasket.

4. A method as claimed in claim 3 in which said gasket is copper, said pressure is substantially 25,000 pounds per square inch, and said gasket is heated to a temperature of about 500°-600° C. at the time said pressure is applied.

#### References Cited by the Examiner

#### UNITED STATES PATENTS

|           |       |                  |          |
|-----------|-------|------------------|----------|
| 2,398,449 | 4/46  | Ronci            | 29-497   |
| 2,818,637 | 1/58  | Roberts          | 29-472.5 |
| 2,965,962 | 12/60 | Ollendorf et al. | 29-470.1 |
| 3,024,519 | 3/62  | Leinkram         | 317-234  |

JOHN F. CAMPBELL, Primary Examiner.